

June 11, 1935.

V. C. ROWE

2,004,394

SELF LIGHTING CIGARETTE

Filed July 2, 1932

FIG. 1



FIG. 2



FIG. 3



FIG. 4



Inventor

V.C. Rowe

By Watson E. Coleman  
Attorney

## UNITED STATES PATENT OFFICE

2,004,394

## SELF LIGHTING CIGARETTE

Victor C. Rowe, Roundup, Mont.

Application July 2, 1932, Serial No. 620,686

3 Claims. (Cl. 131—52)

This invention relates to improvements in cigarettes and pertains particularly to a self-lighting cigarette.

The primary object of the present invention is to provide a cigarette having a tip formed of a substance which will ignite when drawn across a suitable friction surface, so that the cigarette may be readily lighted without the use of matches or any of the other usual lighting devices. 5  
10 Another object of the invention is to provide an improved method of forming a lighting tip upon a cigarette whereby the tip will retain its form and position and whereby the cigarette may be readily grasped to facilitate drawing it across a suitable 15 surface for the production of the necessary friction to effect the ignition of the tip.

A further object of the invention is to provide a method of attaching a lighting tip to a cigarette by means of which the marring of the appearance 20 of the cigarette is prevented and the cigarette is given a distinctive appearance.

The invention will be best understood from a consideration of the following detailed description taken in connection with the accompanying drawing forming part of this specification, with the understanding, however, that the invention is not confined to any strict conformity with the showing of the drawing but may be changed or modified so long as such changes or modifications mark 25 no material departure from the salient features of the invention as expressed in the appended claims.

In the drawing:—

Figure 1 is a view in side elevation of a cigarette formed in accordance with the present invention; 30

Figure 2 is a longitudinal sectional view through the end of a cigarette showing the first step in the formation of the igniting tip thereon; 35

Figure 3 is a longitudinal sectional view of the tip of a cigarette showing the igniting tip applied thereto;

Figure 4 is a perspective view of the bottom portion of a cigarette package showing the scratching surface with which the packet is supplied and over which the tip of the cigarette must be drawn in order to effect its ignition.

Referring now more particularly to the drawing 40 wherein like numerals of reference indicate corresponding parts throughout the several views, the numeral 1 indicates generally a cigarette made in accordance with the present invention, the numeral 2 indicating the ignition tip thereof, while 45 the band-like portion surrounding the cigarette 50

adjacent the ignition tip and indicated by the numeral 3 constitutes a reinforcing area by which the cigarette may be grasped in drawing the same across the scratching surface.

In the manufacture of a cigarette in accordance with the present invention the tip of the same is dipped into or otherwise has applied thereto an aqueous solution of acacia of 30-35% strength. It is preferable that this solution be colored in some suitable manner so as to cover 5 up any discoloration of the paper of the cigarette which may occur from the application of the striking tip material thereto or from the wetting of the tobacco and it is desired that this aqueous solution be colored with a substance such as 10 methylene blue. In addition to providing a distinguishing marking for the cigarette the colored area indicates the portion of the cigarette which should be grasped when lighting the same.

By the use of an aqueous solution of the 20 strength stated there is formed a coating 4 which stiffens the tip of the cigarette and also provides a thin covering 5 over the tobacco in the end thereof. This stiffened portion 4 around the exterior of the cigarette body and the coating 5 is illustrated in an exaggerated manner in Figures 2 and 3 and, as is shown, a slight depression is formed in the end of the cigarette. This depression is brought about by the contraction of the acacia gum as the same dries and there is thus formed in this manner the desired depression for the purpose hereinafter set forth. It will, of course, be understood that in the actual manufacture of the cigarette the coating of 25 acacia gum will be made as thin as possible consistent with the production of the results desired. It is, therefore, desirable that in the application of this coating any excess mucilage be removed from the surface of the paper and from the end of the cigarette after the cigarette end has been 30 dipped or had the mucilage applied thereto in any other manner.

After the tip of the cigarette has been prepared in the manner described it is allowed to 35 partially dry and the striking material is then applied to the tip. The material employed for forming the striking tip is prepared from the following formula.

| Group 1                          | 50    |
|----------------------------------|-------|
| Per cent                         | 50    |
| Potassium chlorate, 48 grains    | 44    |
| Potassium permanganate, 7 grains | 6.5   |
| Copper acetate, 12 grains        | 11    |
| Pumice, 25 grains                | 23 55 |

## Group 2

## Per cent

|                                         |     |
|-----------------------------------------|-----|
| Phosphorous sesquisulfide, 2 grains     | 1.5 |
| Aqueous solution of acacia, (10%) 10 to |     |
| 5 12 cc                                 | 14  |

The above formula is made up as follows:—  
The ingredients of Group 1 are thoroughly mixed together and there is then added to this mixture a sufficiency of the 10% acacia solution set forth in Group 2 to form a thin mucilaginous mixture. The phosphorous sesquisulfide of Group 2 is then added to this mixture and thoroughly incorporated. After allowing the mixture to congeal to a certain extent the remaining portion of the 14% of the 10% acacia solution called for is added and this again brings the mixture to a relatively thin consistency.

The mixture thus prepared is then picked up on a suitable carrier and a drop is allowed to fall upon the end of the cigarette which has been coated with the thicker acacia solution. A drop of sufficient size is employed to just cover the end of the cigarette and make contact with the edge of the paper the drop settling in the depression of which the coating 5 forms the bottom.

When this has dried it will form a rounded tip of the character indicated by the numeral 6. This applied drop of material is then allowed to dry at a moderate temperature. The preferred temperature for drying is 85° F. At this temperature the tip will dry without cracking and will retain its form. After the tip has thoroughly dried the cigarette is ready for use.

While the cigarette tip prepared in accordance with the above formula may be ignited upon a scratching surface of the character provided upon safety match boxes, it is preferred that the package in which the cigarettes may be packed have the bottom thereof coated with a scratching material of the following formula. This scratching surface is indicated by the numeral 7 and the carton to which it is applied is indicated by the numeral 8. The formula for the preferred scratching surface material is as follows:—

|                 |          |
|-----------------|----------|
|                 | Per cent |
| Red phosphorous | 35-50    |
| Litharge        | 10-20    |
| Pumice          | 30-35    |
| Gum solution    | 10-15    |

The surface of the carton is prepared for the application of the material of the above formula by applying a 35% solution of acacia thereto and allowing the same to dry. After mixing the dry ingredients of the formula the gum solution called for is added and the mixture is then applied to the previously prepared surface of the package, by spraying or spreading on with a brush. The gum solution called for in the formula for the scratching surface material is of 35% strength the same as employed in preparing the tip of the cigarette to receive the igniting substance.

A cigarette provided with a tip according to the present invention may be readily ignited in a strong wind or under any other circumstances where the use of a cigarette or mechanical lighter would be difficult and the character of the striking tip is such that no offensive taste or odor will be obtained and the materials employed are non-poisonous in the proportions used.

In addition, the formation of the stiffened area about the tip of the cigarette by the use of the mucilage solution provides a means for grip-

ping the cigarette in lighting the same without danger of tearing the wrapper.

While the formula set forth calls for a mucilage of acacia and the use of a mucilage of acacia has been described for stiffening the end of the cigarette preparatory to applying the igniting material, it is to be understood that the invention is not to be limited to the use of this particular substance for other mucilages may be employed, such for example, as mucilage of 10 tragacanth, however, mucilage of acacia is preferred because of the fact that it is free from unpleasant odor when burned and when dry it provides the correct amount of stiffening particularly where used around the area indicated 15 by the numeral 3. In the making up of the mucilage of acacia it is preferred that it be made according to the method prescribed by the United States pharmacopœia which requires its preparation without the use of heat.

In stating that the tip of the cigarette is allowed to partially dry after the mucilage has been applied thereto it is to be understood that this step is set forth merely for the purpose of making it clear that the complete drying of the 25 tip is not essential to the proper carrying out of the method and that time may be saved by proceeding after partial drying only has taken place.

It is also to be understood that the chemicals 30 must be finely sub-divided as well as thoroughly mixed in order to obtain the best results.

In describing the formation of the striking surface upon the bottom of the cigarette package it was stated that the 35% acacia solution 35 or mucilage is employed. This is preferable but is not absolutely necessary for any other suitable type of mucilage may be used, such for example, as the mucilage which may be bought under the name of Le Pages.

In the mixing of the ingredients of Groups 1 and 2 it was stated that after the addition of a small quantity of the acacia solution and the phosphorous sesquisulfide to the ingredients of Group 1, the mixture is allowed to partially congeal after which the remainder of the required quantity of acacia solution is added. This step is required because of the tendency of the potassium permanganate to reduce to potassium permanganate and manganese oxide when mixed with all of the acacia solution at one time and this reduction is overcome to a certain extent by adding only a portion of the acacia solution and allowing the congealation to partially take place.

Having thus described the invention, what is claimed is:—

1. The method of forming a self-lighting cigarette, which consists in dipping or otherwise impregnating the wrapping at one end of the cigarette and the tobacco exposed at that end into a water solution of acacia gum whereby to form a stiffened area at the end of the cigarette and a slightly hollow reinforcement across the tobacco, drying the gum solution, then placing in said hollow a body of fulminating substance to form a head which does not exceed in diameter the diameter of the stiffened end portion of the cigarette, and finally drying the fulminating substance.

2. The method of manufacturing a self-lighting cigarette which comprises applying a solution of a gum to one end of the cigarette to form a covering for the tobacco in the end of the cigarette and to stiffen the wrapper thereof, then

partly drying the gum solution, the partial drying of the solution causing a contraction of the gum and formation of a hollow in the end of the cigarette, then inserting into the hollow a 5 soft tenacious drop of a fulminating substance and confining the same to the area defined over the end of the cigarette by the partially dried gum solution whereby the side of the cigarette is kept free from said substance and finally completely drying out the gum solution and said substance.

3. The method of forming a self-lighting cigarette, which consists in dipping one end of the cigarette into a water solution of acacia gum of from thirty to thirty-five percent strength 10 to form a covering film across the tobacco at the end of the cigarette and to impregnate the wrap-

ping thereof throughout a portion of the length of the cigarette, then partially drying the dipped end of the cigarette to effect the partial hardening of the gum and the stiffening of the dipped portion of the wrapper, the partial drying of said solution causing contraction of the gum whereby a depression is formed in the end of the cigarette, then applying to the gummed depressed end of the cigarette sufficient of a mixture containing a solution of a gum and chemicals which 15 combine to give a fulminating substance to cover only the end of the cigarette and without perceptibly overlying the sides of the same, and finally drying the gummy mixture of chemicals at an even temperature to form a hard dry tip. 15

VICTOR C. ROWE.